

June 13, 1933.

C. F. SMITH

1,913,688

MANUFACTURE OF FIRE EXTINGUISHERS

Filed Sept. 4, 1931



*Fig. 1.*



*Fig. 2.*



*Fig. 3.*



INVENTOR.

BY *Carlisle F. Smith*  
*Jeffrey, Kimball & Eggleston*  
ATTORNEYS.

## UNITED STATES PATENT OFFICE

CARLISLE F. SMITH, OF ELMIRA, NEW YORK, ASSIGNOR TO AMERICAN-LA FRANCE AND FOAMITE CORPORATION, OF NEW YORK, N. Y., A CORPORATION OF NEW YORK

## MANUFACTURE OF FIRE EXTINGUISHERS

Application filed September 4, 1931. Serial No. 561,133.

The invention refers to an economical process for manufacturing fire extinguishers, and more particularly for connecting the neck ring to the body or shell of the extinguisher. It consists in the successive steps herein described and in the extinguisher resulting therefrom having an improved joint between neck ring and body secured against internal pressure as well as 10 against weakening by corrosion.

Referring to the drawing: Fig. 1 is a central vertical section through the neck ring and the body or shell of the extinguisher showing the parts ready for assembling. Fig. 2 is a view corresponding to Fig. 1 with the ring seated on the shell, and Fig. 3 is a similar view showing the completed joint.

The main shell of the extinguisher marked 20 1 is first provided with a cylindrical projecting rim 2 bossed outwardly therefrom at the top of its dome portion. The shell is then tinned that is coated throughout its entire interior with a coating *a* of solder metal to avoid corrosion by chemicals and this coating is made to extend on to and around and on the outside of the bossed rim. The neck ring 4, cast or forged and provided with an inward flange 5, and having 25 an undercut machined groove 6 on its inner side, is then also coated with solder metal all over as by dipping it, as indicated at *a*. This ring is then externally threaded at 7 and its top surface dressed off to form a gasket seat 8. The coated 30 bossed rim is introduced into it (Fig. 2) and expanded into the undercut groove so as to interlock therewith (Fig. 3). The joint thus formed is then heated so as to 35 fuse the two contiguous coatings and improve the bond of the interlock, at the same time effectually excluding entrance of any of the chemical contents of the extinguisher into the crevice between rim and ring which 40 might corrode and either weaken the joint or produce a leak. A small band of solder 45 may, if desired, be inserted in the depression between the rim and the ring after it has been pressed into place and before heating.

This process of making a fire extinguisher enables the soldering to be done from the outside of the shell rather than through the bottom end of the shell and is advantageous in the particular and specific fire extinguisher art. 55

I claim:

1. The process of making a fire extinguisher which consists in first forming a main shell with an outwardly bossed rim, 60 coating the whole of the interior of the shell and the outside of the rim with solder metal, locating the neck ring exterior to the main shell and bossed rim and expanding such rim into an undercut groove in the inner side of the neck ring, then heating the joint thus formed to fuse the contiguous surfaces thereof. 65

2. The process of making a fire extinguisher which consists in first forming a main shell with an outwardly bossed rim, 70 coating the whole of the interior of the shell and the outside of the rim with solder metal, coating, by dripping, the whole of the neck ring into solder metal, locating the neck ring exterior to the main shell and bossed rim and expanding such rim into an undercut groove in the inner side of the neck ring, then heating the joint thus formed to fuse the contiguous surfaces thereof. 75

3. A fire extinguisher comprising an external neck ring having an inward flange and an undercut internal groove below the flange, a main shell having a bossed rim outwardly bent into interlocking engagement 85 with the undercut groove and having a layer of solder metal intervening between the rim and ring adapted to exclude entrance of chemical into the crevice therebetween and secure against internal pressure. 90

4. The process of making a fire extinguisher which consists in forming a main shell with an outwardly bossed rim, coating said rim outside and inside with solder metal, forming a neck ring having an inward 95 flange and an undercut internal groove below the flange, coating the interior of the ring with solder metal, expanding the bossed rim of the shell outwardly into interlocking engagement with the undercut groove 100

in the neck ring, and then heating the joint thus formed to fuse the solder metal intervening between the rim and ring to exclude entrance of chemical into the crevice therebetween.

5. The process of making a fire extinguisher which consists in first forming a main shell with an outwardly bossed rim, coating the whole of the interior of the 10 shell and the outside of the rim with solder metal, causing the neck ring to seat on the shell exterior to and adjacent the bossed rim and expanding such rim into an undercut groove in the inner side of the neck ring, 15 inserting a band of solder into the depression between the rim and the ring, then heating the joint thus formed to fuse the contiguous surfaces thereof.

In testimony whereof, I have signed this  
20 specification.

CARLISLE F. SMITH.

25

30

35

40

45

50

55

60

65